

May 11, 1943.

L. L. DODGE

2,319,116

PAPER AND METHOD OF MAKING SAME

Filed March 1, 1939



## UNITED STATES PATENT OFFICE

2,319,116

## PAPER AND METHOD OF MAKING SAME

Lloyd L. Dodge, Chicago, Ill., assignor to Rhinelander Paper Company, Rhinelander, Wis., a corporation of Wisconsin

Application March 1, 1939, Serial No. 259,151

8 Claims. (Cl. 92—39)

This invention relates to the preparation of paper having a high degree of transparency, pliability and moistureproofness. More specifically the invention relates to the preparation of paper of enhanced transparency and pliability, that is especially well adapted for use on automatic wrapping and sealing machines.

In my U. S. Patents Nos. 1,992,996, dated March 5, 1935, and 2,099,726, dated November 23, 1937, I have described and claimed methods of preparing a non-greaseproof paper possessing superior qualities over the more expensive greaseproof sheets such as glassine. These patents point out that the greaseproof papers, such as glassine and the like, produced from well hydrated stock, do not have the desired pliability for wrapping papers but possess an inherent springiness when waxed which precludes their satisfactory use on automatic wrapping machines. Such automatic wrapping machines usually fold portions of the waxed paper on itself and seal the fold around the wrapped article by melting the wax on the sheet.

In my Patent No. 1,992,996 a sheet of partially hydrated chemical pulp, preferably sulphite pulp, is formed into a web, dried and plasticized with from 2½ to 10% of a plasticizer such as glycerin, glycols, sugars, deliquescent salts or the like. The plasticized sheet is then supercalendered while in a moist condition. The plasticized and supercalendered sheet can then be waxed.

In my Patent No. 2,099,726 I have described and claimed a method of producing a superior sheet by subjecting the non-greaseproof web, prior to the final waxing operation, to treatment with an aqueous emulsion of wax.

According to the present invention non-greaseproof paper is subjected after supercalendering to a treatment with molten petrolatum or other "amorphous," high-melting hydrocarbon, prior to the final waxing operation. While the particular high melting point hydrocarbons that are preferred for use in the practice of the present invention are here referred to as "amorphous," they are now known to be micro-crystalline waxes. These waxes are produced directly from petroleum by the usual steps of separation customarily practiced in the industry for some years past. The paper, prior to being treated according to this invention, may be plasticized and supercalendered in accordance with the teachings of my patent No. 1,992,996.

The petrolatum used in the method of this invention has a melting point of between 140 and 155° F. Since paraffin waxes seldom have melt-

ing points exceeding 138° F., the petrolatum applied to the sheet prior to the final waxing operation will not bleed through the final wax coating.

5 It is, then, an object of this invention to treat paper with petrolatum or other high-melting amorphous hydrocarbon prior to waxing the paper.

A further object of the invention is to provide 10 a non-greaseproof waxed paper impregnated with petrolatum.

A specific object of the invention is to provide 15 a non-greaseproof, transparent, pliable and moistureproof sheet of paper impregnated with petrolatum and provided with an overlying coating of wax.

Another object of the invention is to use a 20 relatively high melting-point petrolatum for treating a sheet of non-greaseproof paper prior to waxing the sheet.

Other and further objects of the invention will become apparent to those skilled in the art from the following specific example of the process of preparing paper according to this invention.

25 The method of this invention (in a preferred form) is illustrated in the drawing and herein-after more fully described.

On the drawing:

The figure shown is a diagrammatic side elevational view of apparatus suitable for carrying 30 out the method of my invention, with a part thereof shown in section.

A chemical pulp, as for example bleached 35 spruce sulphite pulp or other types of bleached or unbleached sulphite, sulphate or soda pulp, may be used as the furnish to form the paper of this invention. The pulp is beaten only sufficiently to separate and comb out the fibers and to produce a "free stock." The beating operation is terminated before the hydration of the pulp proceeds sufficiently to produce a greaseproof paper.

40 A greaseproof paper may be defined as a paper which resists the penetration of spirits of turpentine for at least one minute. This penetration test is performed by placing a pile of sand of not more than one inch in diameter on the paper to be tested. The sand is covered with sufficient spirits of turpentine to cause the spirits of turpentine to spread outside of the sand pile at least one-eighth inch. A highly enameled book paper is placed beneath the paper being tested. The book paper is examined at intervals until a spot shows on the paper. If the elapsed time 45 for the spot formation on the book paper is over

one minute, the paper being tested is classed as a greaseproof paper.

The non-greaseproof paper intended for use in the method of this invention shows almost instantaneous penetration of the turpentine in a test such as above described, and seldom resists penetration of the turpentine for a period of time exceeding three to five seconds.

The partially hydrated "free" furnish is converted into paper, preferably on a Yankee Four-drinier machine, to form a sheet in which the fibers lie mainly in the direction of travel of the machine. The paper, after being dried on the machine, or during the drying operation, may be treated with 2½ to 10% of plasticizers by weight prior to a supercalendering operation, as is more fully disclosed in my Patent No. 1,992,996 above referred to. Alternatively, the paper can be treated with a wax emulsion prior to the supercalendering operation as is more fully described in my Patent No. 2,099,726 above referred to. If desired, either the plasticizing treatment, the wax emulsion treatment, or both can be omitted.

The method of my invention may be best understood by reference to the accompanying drawing. The paper to be treated, which may be in the form of a mill roll 10, is guided by means of rollers 11 and 12 into contact with the surface of a fountain roll 13, the lower portion of which is immersed in a bath 14 of molten petrolatum. Said petrolatum is contained within a tank 15 provided with heating elements 16, such as steam pipes, for maintaining the petrolatum in a molten condition, preferably at a temperature of from 150 to 175° F. As the fountain roll 13 revolves, it picks up a film of molten petrolatum, the excess of which is doctor off by means of a roll or rod doctor 17. The film of petrolatum remaining on the fountain roll is transferred to the underside of the paper web 18.

The amount of petrolatum transferred to the web 18 may further be controlled by a doctor 19, positioned beyond the fountain roll 13, so that the sheet will not take up more petrolatum than it can retain without causing "bleeding" after the sheet has been waxed. In general, the amount of petrolatum with which the sheet is impregnated should be between 0.5 and 5.0% by weight of the paper, with a preferred range of between 1.5 and 2.5% by weight. As a typical example, if the basis weight of the paper is 21 lbs. per ream of 500 sheets, each 24" x 36", ½ lb. of petrolatum per ream of paper gives excellent results. With heavier or lighter weights of paper, the amount of petrolatum left in the sheet will vary accordingly.

After leaving the fountain roll 13, the web 18 passes around a steam heated roll 20 and a second, larger steam heated roll 21, and thence is guided, as by means of guide rolls 22 and 23, to a rewinder comprising a pair of lower driven rolls 24 and 25 mounted upon a suitable standard 26. The treated paper is wound up on the rewinder into a roll 27. Owing to the speed of travel of the paper, which may be in the neighborhood of 500 feet per minute, the treated paper is still hot, usually in the neighborhood of 150° F., when rewound into the roll 27. Consequently, while the treated paper is in the form of the roll 27, the petrolatum has an opportunity to become thoroughly and uniformly impregnated throughout the entire body of the roll and about the individual fibers of the paper. It is

not necessary to hold the roll 27 for any predetermined period of time before subjecting the petrolatum impregnated paper to a waxing operation, but it may be held for a short period to complete the uniform penetration of the molten petrolatum into the paper web.

After the petrolatum has been thoroughly incorporated into the sheet, the roll is unwound and wet waxed by passing through a molten bath of paraffin wax in accordance with well known practices. Considerably less wax is picked up by the paper, owing to the presence of the petrolatum in the sheet, so that a substantial saving may be effected by virtue of the use of the less expensive petrolatum in place of part of the paraffin wax. Furthermore, only a single waxing step is required, as contrasted with the usual double waxing step commonly employed heretofore.

The petrolatum serves to close up the sheet and impart thereto higher moistureproofness than can be obtained by the use of wax alone. Furthermore, the use of petrolatum gives the sheet greater flexibility and a higher degree of transparency.

By proper control of the amount of petrolatum introduced into the sheet, by the means hereinabove described, the petrolatum will not "bleed," or ooze through the surface coating of wax. A superior wax sheet may thus be prepared at lower cost than can be accomplished without the use of petrolatum.

It will, of course, be understood that various details of construction may be varied through a wide range without departing from the principles of this invention and it is, therefore, not the purpose to limit the patent granted hereon otherwise than necessitated by the scope of the appended claims.

I claim as my invention:

1. In the method of making a waxed non-greaseproof paper of enhanced transparency and pliability from relatively free, partially hydrated stock by successively forming the stock into a paper web having its fibers lying largely in the machine direction, drying, moistening and supercalendering the web, the steps which comprise coating one side of the web with an amorphous petrolatum having a melting point between 140 and 155° F., doctoring off excess petrolatum from the web so as to leave the web impregnated with an amount of said petrolatum insufficient to bleed through the wax, winding the petrolatum treated web into a roll while at a temperature above the melting point of the petrolatum to insure the petrolatum being uniformly fluxed into the web and thereafter applying a coating of paraffin wax to the petrolatum impregnated web.

2. In the method of making waxed non-greaseproof paper of enhanced transparency and pliability from relatively free, only partially hydrated paper stock by forming the stock into a paper web having its fibers lying largely in the machine direction and supercalendering said web, the improvement which comprises coating one side of the web with crude amorphous petrolatum having a melting point of between 140 and 155° F., doctoring off excess petrolatum from the web so that said web contains from 1.5 to 2.5% by weight of petrolatum, winding the petrolatum treated web into a roll while at a temperature above the melting point of the petrolatum and thereafter coating the web with paraffin wax.

3. A sheet of paper impregnated with petrolatum and having a paraffin wax coating overlying the petrolatum impregnated sheet, said

petrolatum having a melting point higher than that of the wax.

4. Wrapping paper suitable for use on automatic wrapping and sealing machines comprising a sheet formed from free chemical pulp stock, said sheet having the fibers thereof lying mainly in one direction, a high melting-point amorphous petrolatum impregnating said sheet and an outer paraffin wax coating thereover, said petrolatum having a melting point higher than that of the wax.

5. A waxed, non-greaseproof paper of enhanced transparency, pliability and moistureproofness comprising a sheet having the fibers thereof lying mainly in one direction and impregnated with amorphous petrolatum and a paraffin wax coating having a lower melting point than the petrolatum covering the sheet, the petrolatum being present in insufficient amount to bleed through said wax coating.

6. In the method of making a relatively transparent, pliable, moisture-proof sheet of waxed paper from relatively free paper stock by successively forming the stock into a paper web having its fibers lying mainly in the machine direction, drying, moistening, and supercalendering the web, the steps which comprise impregnating the web with molten petrolatum having a melting point higher than that of the wax used, regulat-

ing the petrolatum content of the web by doctoring the petrolatum so as to leave the web impregnated with an amount of said petrolatum insufficient to bleed through the wax, and thereafter applying a coating of paraffin wax to the web and over the petrolatum.

7. In the method of making a waxed paper of enhanced transparency and pliability from relatively free paper stock by successively forming the stock into a paper web having its fibers lying mainly in the machine direction, drying, moistening, and supercalendering the web, the steps which comprise coating one side only of the web with molten petrolatum having a melting point higher than that of the wax used, allowing said petrolatum in an amount between 0.5 and 5% by weight of said web to remain on the web, reeling the petrolatum-treated web into a roll while at a temperature above the melting point of the petrolatum to flux the petrolatum into the web, thereafter unreeling the web, and passing the web through a molten paraffin wax bath for waxing the web.

8. A sheet of paper impregnated with from 0.5 to 5% by weight of petrolatum, and a paraffin wax coating overlying the impregnated sheet, said paraffin wax having a lower melting point than the petrolatum.

LLOYD L. DODGE.